

## UNITED STATES PATENT OFFICE

2,228,991

## PRODUCTION OF BRIGHT NICKEL DEPOSIT

Meyer L. Freed, Ansonia, Conn., assignor to The Seymour Manufacturing Co., Seymour, Conn.

No Drawing. Application January 20, 1936,  
Serial No. 59,907

12 Claims. (Cl. 204—14)

This invention relates to an addition agent for nickel plating baths, which causes to be produced on articles plated therein a direct, all-metallic, bright nickel deposit of new and unusual cast, 5 and to the plating process using said agent and the nickel deposit obtained therefrom.

Heretofore, when nickel was deposited from plating solutions of its salts, a dull deposit was obtained on the article plated, which necessitated 10 buffering and polishing the article to give the nickel deposit a bright, glossy, lustrous appearance. In the attempt to obtain this bright, lustrous appearance as a direct result of the plating operation, there have been included in the ordinary nickel electro-plating baths certain addition agents of organic origin, colloidal in character, such as glycerin, gum tragacanth, dextrine, glucose, 15 gum arabic, casein, egg albumin, terpenes, terpene alcohols and aldehydes, natural and synthetic gums and resins and the like, and complex nickel compounds of aromatic sulphonates.

The use of such addition agents is accompanied with serious drawbacks. Extreme care must be observed to avoid any excess of these agents in 25 the plating solution creating great difficulty in the operation of such nickel plating baths. Excesses of these agents void the utility of the bath and even a small excess promotes peeling or cracking of the deposit. Yet methods of analysis 30 are inadequate for accurate and such rigid control of the plating bath composition and are far too cumbersome, time consuming and expensive for practical purposes. Furthermore, due to cataphoresis coupled with capillary action and adsorption, organic material is retained in all of 35 the nickel coatings deposited from plating baths containing such addition agents. As a result, deposits obtained therefrom are not suitably dense, are readily subject to pitting and have reduced 40 resistance to corrosion; are brittle and not suitable for further working. Consequently, such deposits are unsatisfactory as a base deposit to be subsequently covered with chromium plate or with a coating of any other metal.

In addition to the above shortcomings, at their best, deposits produced in the presence of the above addition agents are unattractive as a finish coat by themselves because of their yellowish, white shade.

Likewise, bright nickel coatings that are produced by buffering and polishing are unattractive because of their yellowish hue and also have a tendency to reduce the throwing power of any 50 subsequent deposit of chromium or other metal.

Thus one feature of my invention is the introduction of an addition agent for a nickel plating bath to enable the direct electrodeposition therefrom of an all-metallic bright nickel deposit requiring no buffering or polishing to develop its glossy, lustrous appearance.

A second feature is the development of an addition agent or brightener for a nickel plating bath, the composition and concentration of which agent in the plating bath may be very readily and easily adjusted and determined. 5

Another feature is the direct deposition from a nickel plating bath of a bright, lustrous, hard, ductile, dense, non-porous nickel deposit of any suitable thickness, and exhibiting good adherence and resistance to corrosion and abrasion. 10

A further feature is the addition to a nickel plating bath of an agent that improves the general efficiency of the bath and causes the throwing power of any subsequent deposits of chromium or other metal over the nickel to be increased. 15

Still another feature is the production of a direct bright nickel deposit having a bluish tinge suitable as a final finish in itself or as a suitable base for subsequent deposit of chromium plate. 20

Other objects and features of my invention will occur from the following more detailed description thereof.

In general, my invention consists in the addition to a nickel plating bath of an addition agent 25 comprising a preferably soluble, suitable mixture of a compound of cobalt and a compound of at least one other metal selected from the group consisting of cadmium, zinc and mercury in such relative proportions and in sufficient amount to 30 bring about the deposition from the bath, upon the passage of an electric current from an anode through said bath to a cathode, of a bright nickel deposit upon the cathode, under the particular operating conditions. The addition agent or 35 brightener comprises the mixture of the compound of cobalt and the compound of at least one other metal selected from the group consisting of cadmium, zinc and mercury, either in the solid state or in solution. Whether in the 40 solid form or in solution, the brightener may include, in addition to the suitable combination of the above described metal compounds, other soluble compounds which upon the introduction of the brightener to the plating bath react to 45 assist in anode corrosion, decrease polarization at the anode, increase the conductivity of the bath, prevent the formation of basic compounds and assist in the adjustment of the hydrogen ion concentration of the bath. For brevity in 50 the specification and in the claims, these other soluble compounds will be referred to as "other compounds to effect the plating bath characteristics." It is understood that this general definition shall suffice to include compounds effective 55 for any or all of the purposes herein enumerated.

Particularly satisfactory results are obtained with an addition agent mixture which has for its metallic ion yielding constituents a soluble salt of cobalt and of cadmium. 60

Any soluble cobalt and cadmium, and/or zinc or mercury salts suitable for electroplating may be used in the preparation of my brightener or addition agent, for example, the chlorides or sulfates.

As nickel plating solutions vary in composition, a wide variation in ratio of metallic cobalt constituent in the addition agent to metallic cadmium and/or zinc or mercury constituent is possible. Preferably, the metallic cobalt may be present in from about 99 to about 25 parts thereof to from around 1 to about 75 parts of metallic cadmium and/or zinc or mercury.

Suitable salts for assisting in anode corrosion 15 are ammonium salts, such as the chloride, sulphate, and the like; nickel salts, such as nickel chloride, sulphate and other soluble nickel plating salts. The ammonium salts are also effective in and may be added for decreasing the polarization 20 at the anode and for increasing the conductivity of the plating bath. Nickel chloride and sulphates such as those of sodium and magnesium are also effective for increasing the conductivity of the plating bath.

25 The formation of basic substances may be prevented by including in the addition agent a suitable amount of sulphuric acid.

The addition agent may also contain, for the 30 purpose of assisting in adjusting the hydrogen ion concentration of the plating bath, a suitable quantity of a compound ordinarily added to the bath for such purpose such as boric acid, mineral acid, e. g., sulphuric acid, or an organic acid such as citric acid.

35 I have found that with the more commonly met nickel plating baths, very good results are obtained when there is added thereto a brightener or addition agent which contains any suitable cobalt and cadmium salts in such proportions 40 that the metallic elements are present in the ratio of about 7 1/4 parts cobalt to about 1 part of cadmium. The cadmium may be replaced in whole or in part by zinc and/or mercury in this same ratio to give the same results, as indicated hereinabove.

45 The following examples further illustrate the invention, but the invention is not restricted to these examples:

#### 50 Example 1

A good brightener or addition agent consists of 14.4 parts of commercial crystal cobalt chloride and 1 part of commercial crystal cadmium chloride.

#### 55 Example 2

60 A typical formula for the brightener containing other salts to effect anode corrosion, conductivity, and the pH of the plating bath, and to prevent the formation of basic compounds is:

|                                           | Per cent |
|-------------------------------------------|----------|
| Cobalt chloride (commercial crystal)      | 14       |
| Cadmium chloride (commercial crystal)     | 1        |
| 65 Ammonium chloride (commercial crystal) | 3        |
| Nickel chloride (commercial crystal)      | 7        |
| Sodium sulfate (anhydrous)                | 3        |
| Sulfuric acid                             | 2        |
| Water                                     | 70       |

70 In general, only a small concentration of the brightener according to the present invention in the plating bath is necessary to yield desired results.

75 Examples of typical plating operations and the solutions therefor including my brightener are:

#### Example 3

|                         | Ounces per gal. |
|-------------------------|-----------------|
| Nickel sulfate          | 16              |
| Ammonium chloride       | 3.5             |
| Boric acid              | 3               |
| Brightener of Example 2 | 5/3             |

Such a plating bath has a pH value of 5.6. Operating at about 104° F. under a current density of about 8 amperes per sq. ft., it gives a very satisfactory direct bright nickel deposit. 10

#### Example 4

|                         | Ounces per gal. |
|-------------------------|-----------------|
| Nickel sulfate          | 36              |
| Ammonium chloride       | 3.5             |
| Boric acid              | 3               |
| Brightener of Example 2 | 5/3             |

This plating bath, showing a pH value of 4.4, allows a good, rapid production capacity when operated at a current density around 36 amperes per sq. ft. at a temperature of about 123° F. 20

#### Example 5

Excellent direct bright nickel deposits approaching in color the bluish cast of chromium 25 are obtainable in a good capacity at room temperatures around 70° F. at a current density up to 48 amperes per square foot in a plating bath made up as follows:

|                          | Ounces per gal. |
|--------------------------|-----------------|
| Nickel ammonium sulphate | 12              |
| Nickel sulfate           | 4               |
| Boric acid               | 3               |
| Ammonium chloride        | 4.5             |
| Sodium chloride          | 0.8             |
| Brightener of Example 2  | 0.4             |

having a pH value of 5.5.

The above examples are suitable for adjustment of typical nickel plating baths by addition of my brightener. They are given by way of illustration only and it is not intended to limit the invention thereto. 40

Plating baths, such as shown in the examples, made up initially with the constituents of the brightening addition agents in about the concentrations set forth, may be operated for an extended period depending upon output of plated products without any replenishment of brightener. When, after such extended operation, the deposit obtained appears to be of insufficient 50 brightness, a suitable quantity of brightener may be added to the bath.

However, a nickel plating bath can be operated according to my invention without replenishing the addition agent until the anode is entirely 55 consumed if for the ordinary nickel anode there is substituted a nickel anode containing such proportions of cobalt and at least one other metal selected from the group consisting of cadmium, zinc or mercury as will yield a bright nickel deposit on the cathode. Generally, the proportion of cobalt contained in the anode of my invention is greater than that ordinarily occurring as an impurity in the usual nickel anode.

In plants employing plating baths under other operating conditions as to nickel content, concentration of other ions, hydrogen ion concentration, temperature and current density, the most desirable ratio of cobalt to cadmium and/or zinc or mercury for the conditions may readily be arrived at by a few short experimental test runs easily followed by observation of the changes as the dullness decreases and the proper degree of brightness of the deposit is developed. Thus any nickel plating bath can be readily made up with 75

Such relative proportions and concentrations of the cobalt and cadmium and/or zinc or mercury suitable to yield a bright nickel deposit therefrom under the particular operating conditions observed.

The desired proportions of the brightening agent are very readily controlled by quick, easy and simple methods within the comprehension of the type of help ordinarily employed in a plating plant. Such methods are generally dependent solely on metallic constituents.

By the use of my brightener or addition agent, there is deposited with the nickel small amounts of the other metals, such as, cobalt and cadmium and/or zinc or mercury, the effect of which is to so influence the character of the deposit so that it possesses a direct bright, lustrous appearance requiring no subsequent mechanical treatment. The deposit also has a desirable bluish cast, generally approaching the color of a chromium deposit. It is dense, non-porous, compact, ductile and highly resistant to abrasion and corrosion, and highly adherent.

The type of deposit obtained in accordance with the present invention has a marked tendency to enhance the throwing power of any subsequent deposit of chromium or other metal. Because of its characteristic and unusual color, it is well suitable for use as a finished plate by itself as well as to serve a base coat for a subsequent chromium deposit.

While specific embodiments of my invention have been described for purposes of illustration only, it is to be understood that the invention is not to be restricted thereto, but that it is only to be limited in accordance with the scope of the following claims in the light of the prior art.

1. claim:

1. An aqueous, acid nickel sulfate (selected from the group consisting of nickel sulfate and nickel ammonium sulfate) plating bath, the electrolyte of which comprises in addition to the nickel ions, a brightener consisting of ions of (a) cobalt and of (b) at least one other metal selected from the group consisting of cadmium, zinc and mercury in the proportion approximating about seven and one-quarter parts of cobalt to about one part of the single or combined metals of (b).

2. An aqueous, acid nickel sulfate (selected from the group consisting of nickel sulfate and nickel ammonium sulfate) plating bath, the electrolyte of which comprises in addition to the nickel ions, a brightener consisting of ions of cobalt and of cadmium in the proportion approximating about seven and one-quarter parts of cobalt to about one part of cadmium.

3. An aqueous, acid nickel sulfate (selected from the group consisting of nickel sulfate and nickel ammonium sulfate) plating bath, the electrolyte of which comprises in addition to the nickel ions, a brightener consisting of ions of cobalt and of zinc in the proportion approximating about seven and one-quarter parts of cobalt to about one part of zinc.

4. An aqueous, acid nickel sulfate (selected from the group consisting of nickel sulfate and nickel ammonium sulfate) plating bath, the electrolyte of which comprises in addition to the nickel ions, a brightener consisting of ions of cobalt and of mercury in the proportion approximating about seven and one-quarter parts of cobalt to about one part of mercury.

5. The process of electrodepositing bright

nickel, which comprises passing an electric current from a nickel anode containing cobalt and at least one other metal selected from the group consisting of cadmium, zinc and mercury through an aqueous, acid nickel sulfate (selected from the group consisting of nickel sulfate and nickel ammonium sulfate) plating bath to a cathode, the cobalt and at least one other metal from the group of cadmium, zinc and mercury being present in said nickel anode in such relationship as to be introduced into the bath as a brightening agent and in the proportion approximating about seven and one-quarter parts of cobalt to about one part of the single or combined metals of the group cadmium, zinc and mercury.

6. The process of electrodepositing bright nickel, which comprises passing an electric current from a nickel anode containing cobalt and cadmium through an aqueous, acid nickel sulfate (selected from the group consisting of nickel sulfate and nickel ammonium sulfate) plating bath to a cathode, the cobalt and cadmium being present in said nickel anode in such relationship as to be introduced into the bath as a brightening agent and in the proportion approximating about seven and one-quarter parts of cobalt to about one part of cadmium.

7. The process of electrodepositing bright nickel, which comprises passing an electric current from a nickel anode containing cobalt and zinc through an aqueous, acid nickel sulfate (selected from the group consisting of nickel sulfate and nickel ammonium sulfate) plating bath to a cathode, the cobalt and zinc being present in said nickel anode in such relationship as to be introduced into the bath as a brightening agent and in the proportion approximating about seven and one-quarter parts of cobalt to about one part of zinc.

8. The process of electroplating bright nickel, which comprises passing an electric current from a nickel anode containing cobalt and mercury through an aqueous, acid nickel sulfate (selected from the group consisting of nickel sulfate and nickel ammonium sulfate) plating bath to a cathode, the cobalt and mercury being present in said nickel anode in such relationship as to be introduced into the bath as a brightening agent and in the proportion approximating about seven and one-quarter parts of cobalt to about one part of mercury.

9. The process of electrodepositing bright nickel, which comprises passing an electric current from an anode to a cathode through an aqueous, acid nickel sulfate (selected from the group consisting of nickel sulfate and nickel ammonium sulfate) plating bath in the presence in said bath of a brightener consisting of cobalt ions and ions of at least one other metal selected from the group consisting of cadmium, zinc and mercury in the proportion approximating about seven and one-quarter parts of cobalt to about one part of the single or combined metals of the group of cadmium, zinc and mercury.

10. The process of electrodepositing bright nickel, which comprises passing an electric current from an anode to a cathode through an aqueous, acid nickel sulfate (selected from the group consisting of nickel sulfate and nickel ammonium sulfate) plating bath in the presence in said bath of a brightener consisting of cobalt ions and of cadmium ions in the proportion approximating about seven and one-quarter parts of cobalt to about one part of cadmium.

11. The process of electrodepositing bright

nickel, which comprises passing an electric current from an anode to a cathode through an aqueous, acid nickel sulfate (selected from the group consisting of nickel sulfate and nickel 5 ammonium sulfate) plating bath in the presence in said bath of a brightener consisting of cobalt ions and of zinc ions in the proportion approximating about seven and one-quarter parts of cobalt to about one part of zinc.

10 12. The process of electrodepositing bright

nickel, which comprises passing an electric current from an anode to a cathode through an aqueous, acid nickel sulfate (selected from the group consisting of nickel sulfate and nickel ammonium sulfate) plating bath in the presence 5 in said bath of a brightener consisting of cobalt ions and of mercury ions in the proportion approximating about seven and one-quarter parts of cobalt to about one part of mercury.

MEYER L. FREED. 10